

# United States Patent Office

2,828,205

Patented Mar. 25, 1958

1

2,828,205

## POLYVINYL ACETAL SILVER HALIDE EMULSION CONTAINING POLYVINYL ACETAL COLOR FORMERS

Joseph De Witt Overman, New Brunswick, N. J., assignor to E. I. du Pont de Nemours and Company, Wilmington, Del., a corporation of Delaware

No Drawing. Application June 23, 1953  
Serial No. 363,658

13 Claims. (Cl. 96—74)

This invention pertains to photography and more particularly to a process of preparing color former silver halide dispersions and photographic elements bearing photographic layers of such dispersions. Still more particularly, it pertains to such processes wherein the colloid binding agents for the silver halide grains comprise p-hydroxybenzaldehyde polyvinyl acetals.

In the preparation of multilayer color films utilizing synthetic colloid binding agents for the silver halides, it has been the custom to separately prepare each silver halide emulsion for each respective photographic silver halide emulsion layer. This is inconvenient because it involves a duplication of steps. Thus, a separate operation of grain precipitation and growth, coagulation, washing and redispersion for each of the three emulsions has been practiced. It has been difficult to obtain good sensitometric balance in films made in this manner because the silver halide grains in the respective layers are formed under non-identical conditions.

An object of this invention is to provide a simplified process for the manufacture of differentially sensitized polyvinyl acetal emulsions and emulsion layers for multilayer color films and papers. Another object is to provide a process for the preparation of such emulsions and layers wherein the light-sensitive silver halide grains exhibit similar size distribution in each layer. A further object is to provide a more rapid and efficient manner of preparing the three polyvinyl acetal color forming silver halide emulsions or dispersions for coating multilayer color films. Still other objects will be apparent from the following disclosure.

It has been discovered that p-hydroxybenzaldehyde polyvinyl acetals are excellent protective colloids for silver halide grains and that the aqueous silver halide dispersions made with such colloid binding agents can be ripened to the desired grain size distribution, split into portions and each portion mixed with a polyvinyl acetal color-former, and, if desired, other water-soluble, non-color-forming colloids such as polyvinyl alcohol, partially hydrolyzed polyvinyl acetate, polyvinyl acetals, etc. Two or more of such portions can be mixed with spectral sensitizing dye or dyes and other emulsion adjuvants to produce aqueous coating compositions suitable for coating as cooperative layers on film base or paper and the silver halide grain size distribution and history of treatment of the resulting layers will be essentially the same, thus providing good sensitometric balance in the multilayer photographic element.

The novel process of the invention in its broader aspects comprises precipitating light-sensitive silver halides in an aqueous solution of a p-hydroxybenzaldehyde polyvinyl acetal, allowing the silver halide grains to grow (ripen) to the desired extent, removing the water-soluble salts, if desired, dividing the resulting aqueous dispersion into portions, admixing with respective separated portions a different polyvinyl acetal color-former capable of yielding an azomethine or quinoneimine dye upon color coupling development of the exposed silver halide grains

2

and admixing with at least two of such portions an appropriate spectral sensitizing dye so that the resulting emulsions have strong sensitivity in different primary color regions of the spectrum. The resulting dispersions are admixed with additional p-hydroxybenzaldehyde polyvinyl acetal or other emulsion adjuvants, as desired, such as non-color-forming, water-soluble colloids, to control the emulsion viscosity and the water sensitivity, swelling, thickness, coating weight, etc., of the emulsion layers. For example, the layers may contain from 1/2% to 50% by weight of a water-soluble or hydrophilic polyvinyl alcohol or a partially hydrolyzed polyvinyl ester or a polyvinyl acetal, e. g., the sodium o-sulfo-benzaldehyde acetal of polyvinyl alcohol and p-hydroxybenzaldehyde acetal of polyvinyl alcohol. They are then coated as superimposed layers on a suitable sheet support such as a film base or paper base. A blue light absorbing medium is provided either as a yellow dye or pigment in the blue sensitive layer or as a separate filter layer between the upper blue sensitive layer and the lower layers to prevent blue light from exposing any spectrally sensitized layer.

In a preferred aspect of the invention, a mixture of light-sensitive silver halides are precipitated in an aqueous ethanol solution of a p-hydroxybenzaldehyde polyvinyl acetal colloid, the silver halide grains permitted to ripen, the dispersions of the silver halides in said acetal coagulated, the coagulated dispersion washed free from dissolved inorganic salts, the washed coagulate redissolved in aqueous ethanol and admixed, if desired, with more of said acetal, or other non-color-forming colloid and the resulting solution divided into portions, each portion admixed with an aqueous ethanol solution of a different polyvinyl acetal color former capable of yielding a quinoneimine or azomethine dye upon color-coupling development of exposed silver halide grains, and admixing with two or more of such portions an appropriate spectral sensitizing dye and other emulsion adjuvants respectively, so that the resulting emulsions have strong sensitivity in different primary color regions of the spectrum. The resulting dispersions are then coated as superposed layers on a suitable sheet support such as a film base or paper base.

The p-hydroxybenzaldehyde polyvinyl acetals useful in accordance with the invention are hydrophilic colloids which contain a large number of intralinear vinyl alcohol



units to give them hydrophilic or water-permeable properties. They may also contain a substantial proportion of other acetal groups from aliphatic or aromatic aldehyde-containing carboxylic and/or sulfonic acid groups or their water-soluble salts to increase the water-solubility and/or water permeability of the acetals. The latter aldehydes are, of course, devoid of groups which form color during the color development reaction between silver halide and p-phenylenediamine type color developers. This means that the mixed acetals with p-hydroxybenzaldehyde linkages as well as the simple p-hydroxybenzaldehyde polyvinyl acetals are non-color-forming polyvinyl acetals.

The polyvinyl acetals described in the next preceding paragraph can be prepared by any conventional acetalization reaction from the stated aldehydes or their ethylene glycol or dimethyl or diethyl acetals and an acid catalyst, preferably in an ethylene glycol medium. Suitable procedures are described in Dorough and McQueen U. S. Patent 2,310,943, Martin U. S. Patent 2,513,189, and German Patent 643,650. They can be made from polyvinyl alcohol or partially hydrolyzed polyvinyl esters and hydrolyzed olefine/vinyl acetate copolymers and may con-



parts of polyvinyl alcohol, 18 parts 2-cyanoacetyl-3-phenyl-5-benzofuraldehyde ethylene glycol acetal, and 1 part sodium benzaldehyde-o-sulfonate as described in Martin U. S. patent application S. N. 193,297, filed October 31, 1950, U. S. Patent 2,680,732. The three emulsions are modified by the addition of a sulfur sensitizer; the emulsion containing yellow color former is sensitized to green by the addition of a symmetrical oxycarbocyanine dye and the emulsion containing cyan color forming polymer is sensitized to red light by an unsymmetrical thiocarbocyanine dye which confers no sensitivity in the green region of the spectrum, and the three emulsions are then separately digested and prepared for coating.

A multilayer negative film is then made by coating the three emulsions on 0.005 inch thick cellulose triacetate film base to which have been applied, in order, two thin nitrocellulose layers and an emulsion substratum layer (containing a yellow color-forming polymer of the foregoing type) on one surface and on the other surface a sublayer and a non-halation layer. The green-sensitized, yellow color-forming emulsion is coated directly on the substratum to a silver halide coating weight of 55 mg. per sq. dm. On this emulsion layer is coated a thin separator layer (12 mg. per sq. dm.) of polyvinyl alcohol on which is coated the red-sensitized cyan color-forming emulsion to a silver halide coating weight of 28 mg. per sq. dm. Next, there is applied another thin polyvinyl alcohol separator layer over which is coated the blue-sensitized magenta color-forming emulsion so as to give a silver halide coating weight of 22 mg. per sq. dm.

The completed film is exposed to light from black and white color component positives comprising the blue, green and red records of a multicolor scene and processed to a duplicating color negative as described in the "Journal of the Society of Motion Picture and Television Engineers," November 1950, pp. 455-476.

#### Example II

A redispersed emulsion was prepared at pH 9 and 40 with 30% by weight of ethanol in the aqueous solvent medium as described in Example I but using a polyvinyl acetal prepared with 12 parts of p-hydroxybenzaldehyde and no sodium benzaldehyde-o-sulfonate. This redispersed emulsion was divided into portions, one portion was used in the preparation of a magenta and another in the preparation of a cyan emulsion as described in Example I. The emulsions were coated on separate film bases. The coated films were evaluated by giving them step wedge exposures through appropriate filters on a laboratory sensitometer (non-intermittent intensity scale sensitometer employing a neutral density wedge for modulation of printing light), and the exposed films processed as in Example I, and reading the sensitometric strips so obtained on a precision integrating-sphere densitometer (Frayne, J. G., with Crane, G. R., "Journal of the Society of Motion Picture and Television Engineers," vol. 35, No. 2, August 1950, p. 184) and a modification of this densitometer (A. C. Lapsley and J. P. Weiss, "Journal of the Society of Motion Picture and Television Engineers," vol. 56, January 1951, p. 23). This evaluation demonstrated that the films had satisfactory speed and gamma and satisfactory grain size distribution for use in a color duplicating negative of the type described in Example I.

#### Example III

A redispersed silver halide dispersion is made after the manner described in Example I and is divided into three parts and they are mixed as in that example except that the yellow polyvinyl alcohol acetal color former is made by reacting on a weight basis 100 parts polyvinyl alcohol, 61.5 parts m-benzoylacetamidobenzaldehyde ethylene glycol acetal, and 29 parts sodium benzaldehyde-o-sulfonate. A film is made as in Example I except the polyvinyl alcohol separator layer between the magenta

and cyan layers contains yellow colloidal silver (to augment the filtering of blue light by the tartrazine dye). Evaluation as described in Example I demonstrated that the film had uniform grain size distribution in all layers and good sensitometric balance and was satisfactory as a motion picture color duplicating negative.

A multilayer film is prepared as in Example III with the precipitating and ripening conditions adjusted to give high contrast silver halide. When this film is exposed to appropriately colored light through black and white component negatives comprising the blue, green and red records of a multicolor scene and processed to a color positive as described in the "Journal of the Society of Motion Picture and Television Engineers," November 1950, pp. 455-476, a color positive of excellent color quality is obtained. Alternatively, the film may be exposed to a color negative such as is described in Example I and processed to produce a color print of excellent quality.

#### Example IV

Photographic emulsions are prepared as described in Example I except that they are sensitized and coated as follows: The cyan color-forming emulsion, sensitized to red light, is coated on the treated base so as to give a silver halide coating weight of 50 mg. per sq. dm. On that emulsion is coated a thin layer of polyvinyl alcohol; then the green-sensitized magenta color-forming emulsion is coated over the separator layer so as to give a silver halide coating weight of 23 mg. per sq. dm. Next there is applied another polyvinyl alcohol layer over which is coated the blue sensitive yellow color-forming emulsion (containing tartrazine as a filter dye) so as to give a silver halide coating weight of 22 mg. per sq. dm. Evaluation as described in Example II demonstrated that the complete multilayer film had satisfactory speed, gamma and color balance for use as a motion picture color duplicating negative.

#### Example V

Photographic emulsions are prepared as described in Example I, except that they are sensitized and coated as follows: The magenta color-forming emulsion, sensitized to green light, is coated on the treated triacetate base described above so as to give a silver halide coating weight of 35 mg. per sq. dm. On this emulsion is coated a thin separator layer of polyvinyl alcohol; then the red sensitized cyan color-forming emulsion is coated over the separator layer so as to give a silver halide coating weight of 37 mg. per sq. dm. Next, there is applied another thin separator layer of polyvinyl alcohol over which is coated the blue sensitive yellow color-forming emulsion (containing tartrazine as a filter dye) at a silver bromide coating weight of 35 mg. per sq. dm. Evaluation as described in Example II demonstrated that the complete multilayer film had satisfactory speed, gamma and color balance for use as a motion picture color duplicating negative.

#### Example VI

A redispersed emulsion was prepared at pH 9 and with 28% by weight of ethanol in the aqueous solvent medium as described in Example I but using a polyvinyl acetal prepared with 8 parts of p-hydroxybenzaldehyde and 2 parts of benzaldehyde-o-sodium sulfonate. This redispersed emulsion was used in the preparation of a cyan color-forming emulsion as described in Example I. The resulting emulsion was coated on film base as described in Example I and evaluated as described in Example II. The sensitometric results indicated that the emulsion had satisfactory speed and contrast for use in a duplicating color negative film.

#### Example VII

A redispersed emulsion was prepared at pH 9 and

7  
with 28% by weight of ethanol in the aqueous solvent medium as described in Example I but using a polyvinyl acetal prepared with 10 parts of p-hydroxybenzaldehyde and 4 parts of sodium benzaldehyde o-sulfonate. This redispersed emulsion was used in the preparation of a cyan color-forming emulsion as described in Example I. The resulting emulsion was coated on film base as described in Example I and evaluated as described in Example II. The sensitometric results indicated that the emulsion had satisfactory speed and contrast for use in a duplicating color negative film.

*Example IX*

A redispersed emulsion is prepared as in Example I, using precipitating and ripening conditions adjusted to give high contrast silver bromide. This redispersed emulsion is divided into three parts. One part is mixed with 300 grams per mol of silver of a yellow color-forming polyvinyl acetal made by reacting on a weight basis 100 parts of polyvinyl alcohol, 61.5 parts m-benzoylacetamido benzaldehyde ethylene glycol acetal and 29 parts of sodium benzaldehyde o-sulfonate as described in U. S. Patent 2,513,190, and 200 grams of polyvinyl alcohol; another part is admixed with 300 grams per mol of silver of cyan color-forming polyvinyl acetal made by reacting on a weight basis 100 parts polyvinyl alcohol, 60 parts m-(3-methylsalicylamido)benzaldehyde ethylene glycol acetal and 30 parts sodium benzaldehyde o-sulfonate, as described in U. S. Patent 2,489,655, and with 200 parts of polyvinyl alcohol, while the third part is admixed with 300 grams per mol of silver of a magenta color-forming polyvinyl acetal made by reacting on a weight basis, 100 parts of polyvinyl alcohol, 60 parts of 2-cyanoacetyl-3-phenyl-5-benzofuraldehyde ethylene glycol acetal and 20 parts sodium benzaldehyde o-sulfonate as described in U. S. application Ser. No. 193,297, filed October 31, 1950 now U. S. Patent 2,680,732, and with 200 parts of polyvinyl alcohol. The three emulsions are modified by the addition of a sulfur sensitizer. The emulsion containing the magenta color-former is sensitized to green by the addition of a symmetrical oxycarbocyanine dye and the emulsion containing cyan color-forming polymer is sensitized to red light by an unsymmetrical thiocarbocyanine dye which confers no sensitivity in the green region of the spectrum and the three emulsions are then separately digested and prepared for coating. A multilayer negative film is prepared by coating on a base such as is described in Example I, the red sensitized cyan color-forming emulsion. On this emulsion layer is coated the green sensitized magenta color-forming emulsion and there is next applied a layer of colloidal silver having an optical density to blue light of 1.5, over which there is coated the blue-sensitive yellow color-forming emulsion. The completed film is exposed to light from a color negative having the same conventional layer arrangement of color-former to emulsion sensitivity and processed as described in Example IV to a color-positive of excellent color quality.

The silver halides can be precipitated in the foregoing emulsions in the usual manner by dissolving a soluble, ionizable halide, e. g., sodium, potassium, or ammonium chloride, bromide or iodide, or mixtures thereof in water and by dissolving separately in water a soluble, ionizable silver salt, e. g., silver nitrate, silver sulphamate, silver acetate or silver citrate or mixtures of two or more such compounds. The two solutions are admixed with the solution of simple or mixed p-hydroxybenzaldehyde polyvinyl acetal in any order and in one or several portions depending on the particular photographic qualities desired.

After redispersion of the coagulated silver halide dispersions in the p-hydroxybenzaldehyde polyvinyl acetals the emulsions can be modified before or after addition with the color-forming polyvinyl acetal by the addition of general emulsion sensitizers, e. g., allyl thiourea,

phenyl isothiocyanate, sodium thiosulfate, and allyl isothiocyanate; antifogging agents, e. g., 2-mercaptopbenzothiazole, 1-phenyl-5-mercaptopetrazole, benzatriazole, and 5-nitrobenzimidazole; sensitizing dyes; hardeners, e. g., formaldehyde and other aliphatic aldehydes, dimethylol urea, trimethylol melamine, chrome alum and other chromium compounds or other emulsion adjuvants.

Other water or water-alcohol soluble, non-color-forming colloids such as polyvinyl alcohol, partially hydrolyzed polyvinyl acetate, partially or completely hydrolyzed copolymers of vinyl acetate or acetals of these with aldehydes free of groups which form colored products in the color development reaction, esters or ethers of cellulose or starch, polymers or copolymers of acrylic or methacrylic acid, etc., can be added as desired to improve the solution viscosity, increase the film thickness or improve film permeability. In addition to the solubilizing aldehydes of the examples, other aldehydes containing 10 ionic groups can be used in the polymer, such as o-phthalaldehydic acid, sodium benzaldehyde-m-sulfonate, p-carboxyphenylbenzaldehyde, glyoxylic acid, succinaldehydic acid, adipaldehydic acid, or 3-formylcyclohexaneoic acid can be used. Also, minor amounts of acetal groups prepared from benzaldehyde, acetaldehyde, furfuraldehyde, butyraldehyde, etc. can be included in the polymers as desired to modify the solubility and permeability characteristics.

The p-hydroxybenzaldehyde simple and mixed acetals, used in accordance with the invention, have the desirable 30 property of being halogen acceptors and result in silver halide color-forming emulsions of high speed.

An advantage of this invention is that it provides a simple and practical method of preparing a plurality of silver halide polyvinyl acetal color-forming emulsions. 35 A further advantage is that multilayer papers and films coated from the emulsions have uniform grain size distribution. A further advantage resides in the fact that the multilayer films and papers made from the emulsions have good sensitometric balance. A still further advantage accrues from the economies of operation resulting from the use of a single emulsion formulation for all layers of a multilayer film or paper. Further economies may result from the use of continuous emulsion manufacture techniques.

45 What is claimed is:

1. A process which comprises precipitating light-sensitive silver halides in an aqueous solution of a non-color-forming polyvinyl acetal taken from the group consisting of simple acetals of polyvinyl alcohol with p-hydroxybenzaldehyde and mixed acetals of polyvinyl alcohol with p-hydroxybenzaldehyde and an aldehyde containing a 50 solubilizing group taken from the class consisting of aliphatic and aromatic carboxylic acids and sulfonic acids and their water-soluble salts, the hydroxyl, carboxylic and sulfonic groups being the sole substituent group attached to the hydrocarbon nucleus of said aldehydes, said polyvinyl acetals containing a large number of intralinear  $-\text{CH}_2-\text{CHOH}-$  groups and being hydrophilic in character; allowing the silver halide crystals to ripen and admixing with the dispersion a water-permeable colloid at least a part of which is a polyvinyl acetal color former capable of forming upon color coupling development of an exposed silver salt image a dye taken from the group consisting of quinoneimine and azomethine dyes and containing in one of its tautomeric forms as an integral part of the molecule an active coupling group of the structure



60 70 where X is taken from the group consisting of primary amino, secondary amino and OH groups and n is a number taken from the group consisting of 0 and 1.

2. A process which comprises precipitating light-sensitive silver halides in an aqueous solution of a hydrophilic 75 macromolecular mixed acetal of polyvinyl alcohol with

p-hydroxybenzaldehyde and an aldehyde containing a solubilizing group taken from the class consisting of aliphatic and aromatic carboxylic acids and sulfonic acids and their water-soluble salts, the hydroxyl, carboxylic and sulfonic groups being the sole substituent group attached to the hydrocarbon nucleus of said aldehydes, said polyvinyl acetals containing a large number of intralinear  $-\text{CH}_2-\text{CHOH}-$  groups allowing the silver halide crystals to ripen and admixing with the dispersion a water-permeable colloid at least a part of which is a polyvinyl acetal color former capable of forming upon color coupling development of an exposed silver salt image a dye taken from the group consisting of quinoneimine and azomethine dyes and containing in one of its tautomeric forms as an integral part of the molecule an active coupling group of the structure



where  $X$  is taken from the group consisting of primary amino, secondary amino and OH groups and  $n$  is a number taken from the group consisting of 0 and 1.

3. A process as set forth in claim 2 wherein said aldehyde is sodium benzaldehyde-o-sulfonate.

4. A process which comprises precipitating light-sensitive silver halides in an aqueous solution of a non-color-forming polyvinyl acetal taken from the group consisting of simple acetals of polyvinyl alcohol with p-hydroxybenzaldehyde and mixed acetals of polyvinyl alcohol with p-hydroxybenzaldehyde and an aldehyde containing a solubilizing group taken from the class consisting of aliphatic and aromatic carboxylic acids and sulfonic acids and their water-soluble salts, the hydroxyl, carboxylic and sulfonic groups being the sole substituent group attached to the hydrocarbon nucleus of said aldehydes said polyvinyl acetals containing a large number of intralinear  $-\text{CH}_2-\text{CHOH}-$  groups and being hydrophilic in character; allowing the silver halide crystals to ripen, dividing the resulting aqueous dispersion into portions, and admixing a different polyvinyl acetal color former capable of forming upon color coupling development of an exposed silver salt image a dye taken from the group consisting of quinoneimine and azomethine dyes and containing in one of its tautomeric forms as an integral part of the molecule an active coupling group of the structure



where X is taken from the group consisting of primary amino, secondary amino and OH groups and  $n$  is a number taken from the group consisting of 0 and 1 with each of more than one of such portions.

5. A process which comprises precipitating light-sensitive silver halides in an aqueous solution of a non-color-forming polyvinyl acetal taken from the group consisting of simple acetals of polyvinyl alcohol with p-hydroxybenzaldehyde and mixed acetals of polyvinyl alcohol with p-hydroxybenzaldehyde and an aldehyde containing a solubilizing group taken from the class consisting of aliphatic and aromatic carboxylic acids and sulfonic acids and their water-soluble salts, the hydroxyl, carboxylic and sulfonic groups being the sole substituent group attached to the hydrocarbon nucleus of said aldehydes, said polyvinyl acetals containing a large number of intralinear —CH<sub>2</sub>—CHOH— groups and being hydrophilic in character; allowing the silver halide crystals to ripen, removing the water-soluble salts, dividing the resulting aqueous dispersion into portions, and admixing a different polyvinyl acetal color former capable of forming upon color coupling development of an exposed silver salt image a dye taken from the group consisting of quinoneimine and azomethine dyes and containing in one of its tauto-

meric forms as an integral part of the molecule an active coupling group of the structure.



5 where X is taken from the group consisting of primary amino, secondary amino and OH groups and  $n$  is a number taken from the group consisting of 0 and 1 with each of more than one of such portions.

10 6. A process which comprises precipitating light-sensitive silver halides in an aqueous solution of a non-color-forming polyvinyl acetal taken from the group consisting of simple acetals of polyvinyl alcohol with *p*-hydroxybenzaldehyde and mixed acetals of polyvinyl alcohol with

benzaldehyde and mixed acetals of polyvinyl alcohol with 15 p-hydroxybenzaldehyde and an aldehyde containing a solubilizing group taken from the class consisting of aliphatic and aromatic carboxylic acids and sulfonic acids and their water-soluble salts, the hydroxyl, carboxylic

and their water-soluble salts, the hydroxy, carboxylic and sulfonic groups being the sole substituent group attached to the hydrocarbon nucleus of said aldehydes, said polyvinyl acetals containing a large number of intralinear  $-\text{CH}_2-\text{CHOH}-$  groups and being hydrophilic in character; allowing the silver halide crystals to ripen, dividing the resulting aqueous dispersion into portions, adding a different polyvinyl acetal colloid color former capable of forming upon color coupling development of

capable of influencing upon color coupling development of an exposed silver salt image a dye taken from the group consisting of quinoneimine and azomethine dyes and containing in one of its tautomeric forms as an integral part of the molecule an active coupling group of the structure



35 where X is taken from the group consisting of primary amino, secondary amino and OH groups and n is a number taken from the group consisting of 0 and 1 with each of more than one of such portions, and separately coating the portions as layers on a sheet support.

40 7. A process which comprises precipitating light-sensitive silver halides in an aqueous solution of a non-color-forming polyvinyl acetal taken from the group consisting of simple acetals of polyvinyl alcohol with p-hydroxybenzaldehyde and mixed acetals of polyvinyl alcohol with

45 p-hydroxybenzaldehyde and an aldehyde containing a solubilizing group taken from the class consisting of aliphatic and aromatic carboxylic acids and sulfonic acids and their water-soluble salts, the hydroxyl, carboxylic and sulfonic groups being the sole substituent group at-

50 tached to the hydrocarbon nucleus of said aldehydes, said polyvinyl acetals containing a large number of intra-linear  $-\text{CH}_2-\text{CHOH}-$  groups and being hydrophilic in character; allowing the silver halide crystals to ripen, removing the water-soluble salts, dividing the resulting

55 aqueous dispersion into portions, admixing a different polyvinyl acetal colloid color former capable of forming upon color coupling development of an exposed silver salt image a dye taken from the group consisting of quinone-imine and azomethine dyes and containing in one of its 60 tautomeric forms as an integral part of the molecule an active coupling group of the structure



65 where  $X$  is taken from the group consisting of primary amino, secondary amino and OH groups and  $n$  is a number taken from the group consisting of 0 and 1 with each of more than one of such portions, and separately coating the portions as layers on a sheet support.

70 8. A process which comprises precipitating a mixture of light-sensitive silver halides in an aqueous solution of a non-color-forming polyvinyl acetal taken from the group consisting of simple acetals of polyvinyl alcohol with p-hydroxybenzaldehyde and mixed acetals of polyvinyl alcohol with p-hydroxybenzaldehyde and an aldehyde

75

containing a solubilizing group taken from the class consisting of aliphatic and aromatic carboxylic acids and sulfonic acids and their water-soluble salts, the hydroxyl, carboxylic and sulfonic groups being the sole substituent group attached to the hydrocarbon nucleus of said aldehydes, said polyvinyl acetals containing a large number of intralinear  $-\text{CH}_2-\text{CHOH}-$  groups and being hydrophilic in character; allowing the silver halide crystals to ripen, removing the water-soluble salts, dividing the resulting aqueous dispersion into portions, admixing a different hydrophilic polyvinyl acetal colloid color former capable of forming upon color coupling development of an exposed silver salt image a dye taken from the group consisting of quinoneimine and azomethine dyes and containing in one of its tautomeric forms as an integral part of the molecule an active coupling group of the structure



where X is taken from the group consisting of primary amino, secondary amino and OH groups and n is a number taken from the group consisting of 0 and 1 with each of three of said portions, adding a different spectral photographic sensitizing dye to each of two of such portions, and separately coating the portions as layers on a sheet support.

9. A process as set forth in claim 8 wherein the polyvinyl acetal color formers are respectively capable of forming a dye taken from the group consisting of quinoneimine and azomethine dyes and each color former contains in one of its tautomeric forms as an integral part of the molecule an active coupling group of the structure



where X is taken from the group consisting of primary amino, secondary amino and OH groups and n is a number taken from the group consisting of 0 and 1 and said layers are sensitive to light of three different primary color regions of the spectrum.

10. A process which comprises precipitating a mixture of light-sensitive silver halides in an aqueous solution of a non-color-forming polyvinyl acetal taken from the group consisting of simple acetals of polyvinyl alcohol with p-hydroxybenzaldehyde and mixed acetals of polyvinyl alcohol with p-hydroxybenzaldehyde and an aldehyde containing a solubilizing group taken from the class consisting of aliphatic and aromatic carboxylic acids and sulfonic acids and their water-soluble salts, the hydroxyl, carboxylic and sulfonic groups being the sole substituent group attached to the hydrocarbon nucleus of said aldehydes, said polyvinyl acetals containing a large number of intralinear  $-\text{CH}_2-\text{CHOH}-$  groups and being hydrophilic in character; allowing the silver halide crystals to ripen, dividing the resulting dispersion into portions, admixing an aqueous solution containing a yellow polyvinyl acetal color former with one portion, a magenta polyvinyl acetal color former with another portion and a cyan polyvinyl acetal color former with a third portion, each of said color formers being capable of forming upon color coupling development of an exposed silver salt image a dye taken from the group consisting of quinoneimine and azomethine dyes and containing in one of its tautomeric forms as an integral part of the molecule an active coupling group of the structure



where X is taken from the group consisting of primary amino, secondary amino and OH groups and n is a number taken from the group consisting of 0 and 1, adding a sensitizing dye which confers red but no green sensitivity to one of such emulsions, adding a sensitizing dye which confers green sensitivity to another of such emulsions and coating such emulsions as superposed layers on a support with a yellow light absorbing stratum disposed between the blue-sensitive silver halide emulsion layer and the red and green-sensitive layers.

11. A process as set forth in claim 10 wherein each of said polyvinyl acetal color formers is a mixed acetal having hydrophilic properties and contains acetal groups from sodium benzaldehyde o-sulfonate.

12. A photographic composition comprising an admixture of a dispersion of light-sensitive silver salts in a non-color-forming polyvinyl acetal taken from the group consisting of simple acetals of polyvinyl alcohol with p-hydroxybenzaldehyde and mixed acetals of polyvinyl

20 alcohol with p-hydroxybenzaldehyde and an aldehyde containing a solubilizing group taken from the class consisting of aliphatic and aromatic carboxylic acids and sulfonic acids and their water-soluble salts, the hydroxyl, carboxylic and sulfonic groups being the sole substituent

25 group attached to the hydrocarbon nucleus of said aldehydes, said polyvinyl acetals containing a large number of intralinear  $-\text{CH}_2-\text{CHOH}-$  groups and being hydrophilic in character; and a hydrophilic polyvinyl acetal color former capable of forming upon color coupling

30 development of an exposed silver salt image a dye taken from the group consisting of quinoneimine and azomethine dyes and containing in one of its tautomeric forms as an integral part of the molecule an active coupling group of the structure

35



where X is taken from the group consisting of primary 40 amino, secondary amino and OH groups and n is a number taken from the group consisting of 0 and 1.

13. A composition as set forth in claim 12 wherein each of said polyvinyl acetal color formers is a mixed acetal having hydrophilic properties and containing acetal

45 groups from sodium benzaldehyde o-sulfonate each of said color formers being capable of forming upon color coupling development of an exposed silver salt image a dye taken from the group consisting of quinoneimine and azomethine dyes and containing in one of its tautomeric forms as an integral part of the molecule an active coupling group of the structure

55



where X is taken from the group consisting of primary amino, secondary amino and OH groups and n is a number taken from the group consisting of 0 and 1.

60 References Cited in the file of this patent

## UNITED STATES PATENTS

|              |                |               |
|--------------|----------------|---------------|
| 2,380,032    | Dorough et al. | July 10, 1945 |
| 2,380,033    | Dorough et al. | July 10, 1945 |
| 65 2,534,707 | Glick et al.   | Dec. 19, 1950 |
| 2,538,257    | Martin         | Jan. 16, 1951 |
| 2,599,494    | Sloan          | June 3, 1952  |

U. S. DEPARTMENT OF COMMERCE  
PATENT OFFICE

**CERTIFICATE OF CORRECTION**

Patent No. 2,828,205      Joseph De Witt Overman

March 25, 1958

It is hereby certified that error appears in the printed specification of the above numbered patent requiring correction and that the said Letters Patent should read as corrected below.

Column 2, line 15, for "bezaldehyde" read -- benzaldehyde --; column 3, line 52, for "hydroxyl" read -- hydroxyl --; line 53, for "aminoethyl" read -- aminoethenyl --; column 8, line 3, for "benzatriazole" read -- benzotriazol

Signed and sealed this 27th day of May 1958.

(SEAL)

Attest:

KARL H. AXLINE

Attesting Officer

ROBERT C. WATSON  
Commissioner of Patents